

# United States Patent

[19]

Martin et al.

[11] 3,802,935

[45] Apr. 9, 1974

[54] **DEMAGNETIZATION OF COBALT-RARE EARTH MAGNETS**

[75] Inventors: **Donald L. Martin, Elnora, N.Y.; Rollin J. Parker, Greenville, Mich.**

[73] Assignee: **General Electric Company, Schenectady, N.Y.**

[22] Filed: **May 25, 1972**

[21] Appl. No.: **256,942**

[52] U.S. Cl. .... **148/103, 148/31.57, 148/108**

[51] Int. Cl. .... **H01f 1/02**

[58] Field of Search ..... **148/103, 31.57, 108, 102**

[56] **References Cited**

UNITED STATES PATENTS

|           |        |                     |         |
|-----------|--------|---------------------|---------|
| 3,655,464 | 4/1972 | Benz .....          | 148/103 |
| 2,295,082 | 9/1942 | Jonas .....         | 148/103 |
| 2,837,452 | 6/1958 | De Vos et al. ....  | 148/103 |
| 3,039,891 | 6/1962 | Mitchell.....       | 148/103 |
| 3,102,002 | 8/1963 | Wallace et al. .... | 148/103 |

FOREIGN PATENTS OR APPLICATIONS

858,015 1/1961 Great Britain ..... 148/103

OTHER PUBLICATIONS

Bozorth, R. M.; "Ferromagnetism," New York, 1951,

pp. 344, and 713-714.

Buschow, K. et al.; "Permanent Mag. Materials of Re-Co Compounds," in "Zeit. Furr Physik," 26, 1969, pp. 157-160.

Primary Examiner—Hyland Bizot

Assistant Examiner—W. R. Satterfield

Attorney, Agent, or Firm—Jane M. Binkowski; Joseph T. Cohen; Jerome C. Squillaro

[57] **ABSTRACT**

A cobalt-rare earth intermetallic permanent magnet having a high intrinsic coercive force is substantially or completely demagnetized by low energy means. The magnet is heated to an elevated temperature ranging from 40 to 75 percent of its Curie temperature. At such temperature it is demagnetized and the extent of this demagnetization depends largely on the specific temperature to which the magnet is heated and its self-demagnetizing field. If necessary, an external demagnetizing field, which is at least 50 percent below the magnet's intrinsic coercive force at room temperature, is applied to the magnet at the elevated temperature to attain substantial or complete demagnetization.

**4 Claims, No Drawings**

## DEMAGNETIZATION OF COBALT-RARE EARTH MAGNETS

The present invention relates generally to the art of demagnetizing cobalt-rare earth permanent magnets. In one aspect, it relates to the use of reduced energy means to demagnetize a cobalt-rare earth permanent magnet without significantly deteriorating its magnetic properties, i.e., these properties being substantially or completely recoverable by remagnetization.

Permanent magnets, i.e., "hard" magnetic materials such as the cobalt-rare earth intermetallic compounds, are of technological importance because they can maintain a high, constant magnetic flux in the absence of an exciting magnetic field or electrical current to bring about such a field.

Within the past few years a new class of materials for making permanent magnets has been developed, based on cobalt and rare-earth elements. The improvement over prior art materials is so great that the cobalt-rare-earth magnets stand in a class by themselves. In terms of their resistance to demagnetization the new materials are from 20 to 50 times superior to conventional magnets of the Anico type, and their magnetic energy is from two to six times greater. Since the more powerful the magnet for a given size is the smaller it can be for a given job, the cobalt-rare-earth magnets have applications for which prior art materials cannot even be considered.

Demagnetization of cobalt-rare earth permanent magnets is frequently required as a part of the manufacturing process for example, shipping the magnet in the demagnetized condition is advantageous.

The high intrinsic coercive force  $H_{ci}$  of the cobalt-rare earth magnets makes it difficult to demagnetize them by normal means such as an a/c field. Demagnetization of Alnico or BaO ferrite is readily accomplished by a 2,500 - 3,000 a/c field; however, such a field is too low for most of the cobalt-rare earth permanent magnets where the  $H_{ci}$  value may exceed 15,000 oersteds at room temperature. The energy requirements for furnishing the necessary demagnetizing field for these cobalt-rare earth magnets are too high to be practical.

The Curie temperature is the temperature above which a magnetic material loses its magnetic properties. For most cobalt-rare earth magnets, the Curie temperature generally ranges from about 500°C to 735°C and for some it may be as low as about 375°C. Thermal demagnetization by heating above the Curie temperature is inconvenient for commercial use because of the danger of permanently deteriorating the magnetic properties by this additional high temperature heat treatment.

Briefly stated, the present process comprises providing a cobalt-rare earth intermetallic magnet having an intrinsic coercive force higher than 5,000 oersteds, heating said magnet to an elevated temperature ranging from 40 to 75 percent of its Curie temperature. Then, if necessary to attain substantial or complete demagnetization of the magnet, applying to the magnet at elevated temperature a demagnetizing field which is at least 50 percent below the magnet's intrinsic coercive force  $H_{ci}$  at room temperature. The magnet is then preferably cooled to room temperature. The rate of cooling of the magnet is not critical.

The present process is particularly useful for cobalt-rare magnets having at room temperature an intrinsic

coercive force  $H_{ci}$  in excess of 5,000 oersteds. Specifically, when a permanent magnet material is magnetized, a magnetization value of  $4\pi J$  gauss is established therein. The shape of the magnet imposes a self-demagnetizing field of  $H$  oersteds. Together, these properties,  $4\pi J$  and the self-demagnetizing field  $H$  equal the operating flux density or open circuit induction  $B_o$  which is also measured in gauss. The intrinsic coercive force  $H_{ci}$  of the permanent magnet is the value of the external demagnetizing field which must be applied to the magnet at room temperature to reduce its magnetization  $4\pi J$  to zero.  $H_{ci}$  is a measure of a permanent magnet's resistance to demagnetization.

Cobalt-rare earth magnets having an intrinsic coercive force in excess of 5,000 oersteds are particularly useful in the present process. Such magnets are usually sintered cobalt-rare earth intermetallic products which may be prepared by a number of techniques. Briefly, the cobalt-rare earth intermetallic material is formed and converted to particulate form. The particles are compressed into a green body which is then sintered in a substantially inert atmosphere to produce a sintered body of the desired density.

Cobalt-rare earth intermetallic compounds exist in a variety of phases, but the  $Co_5R$  intermetallic single phase compounds (in each occurrence R designates a rare earth metal) have exhibited the best magnetic properties, and generally, sintered products composed of the  $Co_5R$  phase or containing the  $Co_5R$  phase in at least a significant amount have produced the best permanent magnets.

Specifically, the present invention is particularly useful for the sintered cobalt-rare earth permanent magnets disclosed in U.S. Pat. No. 3,655,464, U.S. Pat. No. 3,655,463 and copending Ser. No. 33,224, now U.S. Pat. No. 3,695,945, all filed on Apr. 30, 1970 in the name of Mark G. Benz, and assigned to the assignee hereof, and all of which by reference are made part of the disclosure of the present application.

Each of the aforementioned patents and patent application discloses a process for preparing novel sintered cobalt-rare earth intermetallic products which can be magnetized to form magnets having improved permanent magnet properties.

Briefly stated, in U.S. Pat. No. 3,655,464 a particulate mixture of a base Co-R alloy and an additive Co-R alloy, where R is a rare earth metal or metals is sintered to produce a product having a composition lying outside the  $Co_5R$  single phase on the rare earth richer side. Specifically, the base alloy is one which at sintering temperature exists as a solid  $Co_5R$  intermetallic single phase. Since the  $Co_5R$  single phase may vary in composition, the base alloy may vary in composition which can be determined from the phase diagram for the particular cobalt-rare earth system, or empirically. The additive cobalt-rare earth alloy is richer in rare earth metal than the base alloy and at sintering temperature it is at least partly in liquid form and thus increases the sintering rate. The additive alloy may vary in composition and can be determined from the phase diagram for the particular cobalt-rare earth system or it can be determined empirically.

The base and additive alloy, in particulate form, are each used in an amount to form a mixture which has a cobalt and rare earth metal content substantially corresponding to that of the final desired sintered product since sintering causes little or no loss of these compo-

nents. The additive alloy should be used in an amount sufficient to promote sintering, and generally, should be used in an amount of at least 0.5 percent by weight of the base-additive alloy mixture. The particulate mixture is compressed into a green body of the desired size and density. Preferably, the particles are magnetically aligned along their easy axis prior to or during compression since the greater their magnetic alignment, the better are the resulting magnetic properties.

The green body is sintered in a substantially inert atmosphere to produce a sintered body of desired density. Preferably, the green body is sintered to produce a sintered body wherein the pores are substantially non-interconnecting, which generally is a sintered body having a density of at least about 87 percent of theoretical. Such non-interconnectivity stabilizes the permanent magnet properties of the product because the interior of the sintered product or magnet is protected against exposure to the ambient atmosphere.

Sintering temperature depends largely on the particular cobalt-rare earth intermetallic material to be sintered, but it must be sufficiently high to coalesce the component particles. Preferably, sintering is carried out so that the pores in the sintered product are substantially non-interconnecting. For cobalt-samarium alloys, as well as most cobalt-rare earth alloys, a sintering temperature ranging from about 950°C to about 1,200°C is suitable. Specifically, for cobalt-samarium alloys a sintering temperature of 1,100°C is particularly satisfactory.

The density of the sintered product may vary. The particular density depends largely on the particular permanent magnet properties desired. Preferably, to obtain a product with substantially stable permanent magnet properties, the density of the sintered product should be one wherein the pores are substantially non-interconnecting and this occurs usually at a density or packing of about 87 percent. Generally, for a number of applications, the density of the sintered product may range from about 80 percent to 100 percent. For example, for low temperature applications, a sintered body having a density ranging down to about 80 percent may be satisfactory.

The procedure for forming sintered products disclosed in U.S. Pat. No. 3,655,463 is substantially the same as that disclosed in U.S. Pat. No. 3,655,464 except that an additive Co-R alloy which is solid at sintering temperature and which is richer in rare earth metal than the base alloy is used.

The procedure for forming the sintered products disclosed in U.S. Pat. application Ser. No. 33,224 now U.S. Pat. No. 3,695,945 is substantially the same as that disclosed in U.S. Pat. No. 3,655,464 except that a cobalt-rare earth metal alloy of proper composition is initially formed.

When used in the present process, the sintered products of the referred to U.S. patents and copending patent application contain a major amount of the  $Co_5R$  solid intermetallic phase, generally at least about 70 percent by weight of the product, and a second solid Co-R intermetallic phase which is richer in rare earth metal content than the  $Co_5R$  phase and which is present in an amount of up to about 30 percent by weight of the product. Traces of other cobalt-rare earth intermetallic phases, in most instances less than one percent by weight of the product, may also be present.

In addition, copending U.S. Pat. application Ser. No. 86,288 now U.S. Pat. No. 3,684,593 entitled "Heat-Aged Sintered Cobalt-Rare Earth Intermetallic Product And Process", filed on Nov. 2, 1970 in the names of Mark G. Benz and Donald L. Martin and assigned to the assignee hereof, is, by reference, made part of the disclosure of the present application. Briefly stated, in U.S. Ser. No. 86,288 now U.S. Pat. No. 3,684,593 there is disclosed a process for preparing heat-aged 10 novel sintered cobalt-rare earth intermetallic products by providing a sintered cobalt-rare earth intermetallic product ranging in composition from a single solid  $Co_5R$  phase to that composed of  $Co_5R$  phase and a second phase of solid Co-R in an amount of up to about 15 30 percent by weight of the product and richer in rare earth metal content than said  $Co_5R$ , and heat-aging said product at an aging temperature within 400°C below the temperature at which it was sintered to precipitate Co-R phase richer in rare earth metal content than said 20  $Co_5R$  in an amount sufficient to increase intrinsic and/or normal coercive force of said product by at least 10 percent, where R is a rare earth metal or metals. Heat-aging is carried out in an atmosphere such as argon in which the material is substantially inert. The precipitated Co-R phase is generally present in an amount ranging from about 1 to 15 percent by weight of the product. The present invention is particularly useful for these heat-aged sintered products.

The rare earth metals useful in preparing the cobalt-rare earth alloys and intermetallic compounds used in forming the sintered products are the 15 elements of the lanthanide series having atomic numbers 57 to 71 inclusive. The element yttrium (atomic number 39) is commonly included in this group of metals and, in this 35 specification, is considered a rare earth metal. A plurality of rare earth metals can also be used to form the present desired cobalt-rare earth alloys or intermetallic compounds which, for example may be ternary, quaternary or which may contain an even greater number of 40 rare earth metals as desired.

Representative of the cobalt-rare earth alloys useful in forming the sintered products are cobalt-cerium, cobalt-praseodymium, cobalt-neodymium, cobalt-promethium, cobalt-samarium, cobalt-europium, cobalt-gadolinium, cobalt-terbium, cobalt-dysprosium, cobalt-holmium, cobalt-erbium, cobalt-thulium, cobalt-ytterbium, cobalt-lutecium, cobalt-yttrium, cobalt-lanthanum and cobalt-misch metal. Misch metal is the most common alloy of the rare earth metals which contains the metals in the approximate ratio in which they occur in their most common naturally occurring ores. Examples of specific ternary alloys include cobalt-samarium-misch metal, cobalt-cerium-praseodymium, cobalt-yttrium-praseodymium, and cobalt-praseodymium-misch metal.

In carrying out the present process, the permanent magnet is heated to an elevated temperature which ranges from 40 to 75 percent of its Curie temperature. The higher the temperature within this specified range, the greater is the extent to which the magnet is demagnetized. The Curie temperature for a particular material is readily available in the art. Specifically, for the  $Co_5Sm$  intermetallic compound it is 725°C, for  $Co_5Pr$  it is 610°C, for  $Co_5La$  it is 570°C, for  $Co_5Gd$  it is 735°C, for  $Co_5Mischnetal$  it is 500°C and for  $Co_5Ce$  it is 375°C. Heating the magnet to the elevated temperature can be carried out in air if such heating does not signifi-

cantly oxidize the material. Preferably, the permanent magnet is heated in an atmosphere in which it is substantially inert such as argon. In the present invention, the magnet need only be brought up to the elevated temperature and the period of time which it is at temperature is not critical.

The extent to which the magnet is demagnetized at the present elevated temperature depends largely on the specific temperature to which it is heated and its self-demagnetizing field which is determined by its shape. Specifically, when the magnet is small and has a low effective  $l/d$  ratio, where  $l$  is length and  $d$  is the diameter, for example if it is a cylindrical bar having a low  $l/d$  ratio such as one or less than one, it has a high self-demagnetizing field. Heating such a magnet to a temperature which is 40 to 75 percent of its Curie temperature is ordinarily sufficient to substantially or completely demagnetize it. By substantial demagnetization it is meant that the open circuit induction  $B_o$  of the magnet has been decreased by at least about 80 percent.

As the  $l/d$  ratio of the magnet increases, its self-demagnetizing field decreases. For magnets having a high  $l/d$  ratio, such as greater than one, the present heat treatment alone may not substantially or completely demagnetize the magnet. In such instance, to attain substantial or complete demagnetization of the magnet, it is heated to an elevated temperature which is 40 to 75 percent of its Curie temperature, and at this elevated temperature, an external demagnetizing field is applied to the magnet which is at least 50 percent below the magnet's intrinsic coercive force  $H_{ci}$  at room temperature.

The external demagnetizing field can be produced by a DC or AC field provided by means such as an AC solenoid or electromagnet or even by a permanent magnet.

Alternatively, where the cobalt-rare earth permanent magnet is substantially or completely demagnetized by heating it to a temperature only in the upper portion of the temperature ranging from 40 to 75 percent of its Curie temperature, it may be desirable to heat it to a temperature in the lower portion of this temperature range and attain substantial demagnetization by applying the said demagnetizing field to the magnet at such lower temperature range.

As a result of the present process, cobalt-rare earth permanent magnets are demagnetized without significant deterioration of their permanent magnet properties. Specifically, the permanent magnet properties of the cobalt-rare earth magnets demagnetized in accordance with the present process are substantially or completely recoverable by remagnetization of the magnet.

All parts and percentages used herein are by weight unless otherwise noted.

The invention is further illustrated by the following

examples in which, unless otherwise noted, the conditions and procedure were as follows:

The magnetizing field was used to magnetically align along the easy axis.

All sintering was carried out in an inert atmosphere of purified argon and upon completion of the sintering, the sintered product was cooled in the same purified argon atmosphere.

The density of the sintered product is given as packing. Packing is the relative density of the material, i.e., it is a percent of theoretical. Packing was determined by a standard method using the following equation:

$$\frac{\text{Weight}}{\text{Volume}} \times 100 = \% \text{ Packing}$$

$$\frac{8.6 \text{ g/cc.}}{}$$

where 8.6g/cc. is the density of  $\text{Co}_5\text{Sm}$ .

#### EXAMPLE

In the runs of the following table, each alloy melt was made under purified argon by induction melting and cast into an ingot. The ingot was then crushed in air by means of mortar and pestle or in a jaw crusher in nitrogen and then ground in nitrogen by fluid energy milling into a powder of 6 to 8 microns average particle size. An additive alloy was admixed with a base alloy by tumbling to form a substantially thorough mixture which was stable since the additive was substantially non-reactive in air and was slightly magnetic. In the runs of the following table, the composition of the base alloy was 68 percent cobalt-32 percent samarium, the composition of the additive alloy was 40 percent cobalt-60 percent samarium, and the base and additive alloys were each used in an amount to give a composition of 63.1 percent cobalt-36.9 percent samarium.

The green body of each run was formed by packing the mixture into a rubber tube having a working space of  $3/8$  inch in diameter and  $1 \frac{3}{4}$  inch long. The tube was placed in an axial magnetic field of 60,000 oersteds to align the particles along the easy axis. After aligning, the powder was compressed and the sample was subsequently hydrostatically pressed under 200,000 psi. The pressed samples, i.e., green bodies, had a packing density of about 80 percent. The green bodies were cylindrical bars. Generally, the green bodies were machined to make a right cylinder of proper dimensions for testing purposes.

The green bodies were then sintered. In Run Nos. 1, 3 and 4, the green body was sintered for 1 hour at  $1,120^\circ\text{C}$ ; furnace cooled to  $875^\circ\text{C}$  and held at  $875^\circ\text{C}$  for  $\frac{1}{2}$  hour. In Run No. 2, the sintered product was prepared in the same manner as in Run No. 1 except that sintering temperature was  $1,115^\circ\text{C}$ . The sintered products contained the  $\text{Co}_5\text{Sm}$  phase in an amount of about 94 percent. The resulting sintered products were then magnetized and demagnetized as shown in the following table.

| Run No. | Packing (%) | length/diameter | Permanent Magnet Treatment                                                                                                                                                                                                                           | Properties                           |                                              |
|---------|-------------|-----------------|------------------------------------------------------------------------------------------------------------------------------------------------------------------------------------------------------------------------------------------------------|--------------------------------------|----------------------------------------------|
|         |             |                 |                                                                                                                                                                                                                                                      | Open Circuit Induction $B_o$ (gauss) | Intrinsic Coercive Force $H_{ci}$ (oersteds) |
| 1       | 95          | 4.45            | (a) After magnetization in 60,000 oersteds at room temperature<br>(b) Heated to $400^\circ\text{C}$ for 30 minutes, demagnetizing field of about $-650$ oersteds applied by AC field at $400^\circ\text{C}$ and then air cooled to room temperature. | 9290<br>8400                         | 18,700                                       |
| 5       |             |                 |                                                                                                                                                                                                                                                      |                                      |                                              |

| Run No. | Packing (%) | length/diameter | Permanent Magnet Treatment                                                                                                                                                                                       | Properties                           |                                           |
|---------|-------------|-----------------|------------------------------------------------------------------------------------------------------------------------------------------------------------------------------------------------------------------|--------------------------------------|-------------------------------------------|
|         |             |                 |                                                                                                                                                                                                                  | Open Circuit Induction $B_o$ (gauss) | Intrinsic Coercive Force $H_c$ (oersteds) |
|         |             |                 | (c) After magnetization in 60,000 oersteds at room temperature, heated to 425°C for 30 minutes, demagnetizing field of about -650 oersteds applied by AC field at 425°C and then air cooled to room temperature. | 5700                                 |                                           |
|         |             |                 | (d) After magnetization in 60,000 oersteds at room temperature, heated to 475°C for 30 minutes, demagnetizing field of about -650 oersteds applied by AC field at 475°C and then air cooled to room temperature. | 1500                                 |                                           |
|         |             |                 | (e) After magnetization in 60,000 oersteds at room temperature, heated to 525°C for 30 minutes, demagnetizing field of about -650 oersteds applied by AC field at 525°C and then air cooled to room temperature. | 0                                    |                                           |
|         |             |                 | (f) After magnetization in 60,000 oersteds at room temperature.                                                                                                                                                  | 9150                                 |                                           |
|         |             |                 | (g) Heated to 400°C for 30 minutes and air cooled to room temperature.                                                                                                                                           | 9140                                 |                                           |
|         |             |                 | (h) After magnetization in 60,000 oersteds at room temperature, heated to 425°C for 30 minutes and air cooled to room temperature.                                                                               | 8190                                 |                                           |
|         |             |                 | (i) After magnetization in 60,000 oersteds at room temperature, heated to 475°C for 30 minutes and air cooled to room temperature.                                                                               | 3050                                 |                                           |
|         |             |                 | (j) After magnetization in 60,000 oersteds at room temperature.                                                                                                                                                  | 9130                                 |                                           |
| 2       | 93          | 4.2             | (a) After magnetization in 60,000 oersteds at room temperature.                                                                                                                                                  | 8910                                 | 20,800                                    |
|         |             |                 | (b) Heated to 425°C for 30 minutes and air cooled to room temperature.                                                                                                                                           | 8660                                 |                                           |
|         |             |                 | (c) After magnetization in 60,000 oersteds at room temperature, heated to 425°C for 30 minutes, demagnetizing field of about -650 oersteds applied by AC field at 425°C and then air cooled to room temperature. | 1175                                 |                                           |
|         |             |                 | (d) After magnetization in 60,000 oersteds at room temperature, heated to 425°C for 30 minutes, demagnetizing field of about -800 oersteds applied by DC field at 425°C and then air cooled to room temperature. | 55                                   |                                           |
|         |             |                 | (e) After magnetization in 60,000 oersteds at room temperature.                                                                                                                                                  | 8870                                 |                                           |
| 3       | 90          | 3.56            | (a) After magnetization in 60,000 oersteds at room temperature.                                                                                                                                                  | 8520                                 | 22,900                                    |
|         |             |                 | (b) Heated to 500°C for 30 minutes and air cooled to room temperature.                                                                                                                                           | 2280                                 |                                           |
|         |             |                 | (c) After magnetization in 60,000 oersteds at room temperature.                                                                                                                                                  | 8260                                 |                                           |
| 4       | 90          | 0.61            | (a) After magnetization in 60,000 oersteds at room temperature.                                                                                                                                                  | 5000                                 | 22,900                                    |
|         |             |                 | (b) Heated to 500°C for 30 minutes and air cooled to room temperature.                                                                                                                                           | 190                                  |                                           |
|         |             |                 | (c) After magnetization in 60,000 oersteds at room temperature.                                                                                                                                                  | 4990                                 |                                           |

The runs in the table illustrate the present invention. Run No. 1, steps (b) to (e) show that by heating to temperature and applying a relatively small demagnetizing field at temperature, the permanent magnet is substantially or completely demagnetized as illustrated by the open circuit induction which is decreased significantly or reduced to zero. Step (f) shows that the open circuit induction is substantially recoverable upon remagnetization. On the other hand, Run No. 1, steps (g) to (i) show the extent to which certain elevated temperatures alone demagnetize the permanent magnet as illustrated by the reduction in its open circuit induction  $B_o$ . Step (j) shows that the open circuit induction is substantially recoverable upon remagnetization of the magnet.

Run No. 2 shows the significant decrease in open circuit induction which can be attained by heating to temperature and applying a relatively small demagnetizing field in accordance with the present invention.

In Run No. 4 heating to temperature alone was sufficient to substantially demagnetize the permanent mag-

net since this magnet had a low  $1/d$  ratio, and therefore, a high self-demagnetizing field.

What we claim as new and desire to secure by Letters Patent of the United States is:

1. A process for treating a cobalt-rare earth permanent magnet to demagnetize said magnet to decrease its open circuit induction  $B_o$  by at least 80 percent so that said open circuit induction  $B_o$  is substantially or completely recoverable by remagnetization of said magnet, said magnet having a length to diameter ratio of one or less than one and an intrinsic coercive force in excess of 5,000 oersteds and said magnet being a sintered product wherein the pores are substantially non-interconnecting and having a density ranging from about 87 to 100 percent and consisting essentially of compacted particulate alloy consisting essentially of a composition ranging from a single solid  $Co_5R$  phase to a  $Co_5R$  phase and a second solid Co-R phase in an amount up to about 30 percent by weight of said product and richer in rare earth metal content than said

$\text{Co}_5\text{R}$  phase, where  $\text{R}$  is a rare earth metal or metals, which comprises bringing said magnet up to an elevated temperature ranging from 40 to 75 percent of its Curie temperature in an atmosphere in which said magnet is not significantly oxidized and cooling said magnet to room temperature.

2. A process according to claim 1 wherein  $\text{R}$  is samarium.

3. A process for treating a cobalt-rare earth permanent magnet to demagnetize said magnet to decrease its open circuit induction  $B_o$  by at least 80 percent so that said open circuit induction  $B_o$  is substantially or completely recoverable by remagnetization of said magnet, said magnet having a length to diameter ratio greater than one and an intrinsic coercive force in excess of 5,000 oersteds and said magnet being a sintered product wherein the pores are substantially non-interconnecting and having a density ranging from

about 87 to 100 percent and consisting essentially of compacted particulate alloy consisting essentially of a composition ranging from a single solid  $\text{Co}_5\text{R}$  phase to a  $\text{Co}_5\text{R}$  phase and a second solid Co-R phase in an amount up to about 30 percent by weight of said product and richer in rare earth metal content than said  $\text{Co}_5\text{R}$  phase, where  $\text{R}$  is a rare earth metal or metals, which comprises bringing said magnet up to an elevated temperature ranging from 40 to 75 percent of its Curie temperature in an atmosphere in which said magnet is not significantly oxidized, applying to said magnet at said elevated temperature an external demagnetizing field having a maximum value which is at least 50 percent below the intrinsic coercive force of said magnet and cooling said magnet to room temperature.

4. A process according to claim 3 wherein  $\text{R}$  is samarium.

20

\* \* \* \* \*

25

30

35

40

45

50

55

60

65